

## United States Patent Office

3,434,795

Patented Mar. 25, 1969

1

3,434,795

## METHODS OF PROCESSING WOOL AND OTHER HAIR FIBERS

Alton A. Cook, Bloomfield, and Ira Sapers, Newark, N.J., assignors to Arkansas Company, Inc., Newark, N.J., a corporation of New York

No Drawing. Filed Dec. 28, 1965, Ser. No. 517,138  
Int. Cl. D06m 3/02

U.S. Cl. 8—127.6

6 Claims

## ABSTRACT OF THE DISCLOSURE

The present invention relates to the wet processing of wool and other hair fibers in the presence of an hydroxylamine salt of a strong mineral acid, for the purpose of eliminating the natural yellowish cast characteristic of such fibers which often become more pronounced in high temperature dyeing procedures and in processing such fibers under alkaline conditions.

This invention relates to methods of processing wool and other hair fibers and to hair fibers treated by such methods. The invention is particularly concerned with the wet processing of hair fibers.

It is a matter of general knowledge that all hair fibers, whether their origin be sheep, camels, goats or other animals, possess to a greater or lesser extent a yellowish cast or coloration when they are removed from the body of the animal and initially processed. This yellowish cast becomes more pronounced during high temperature dyeing procedures, particularly when the dyeing temperatures are in the range of 200° F. to 212° F. Yellowing also increases when the hair fibers are subjected to alkaline processing, particularly when the processing takes place at temperatures above 190° F.

Conventional reducing agents, such as sodium bisulfite, sodium or zinc formaldehyde sulfoxylate, or sodium or zinc hydrosulfite, lighten the wool, but this effect is only temporary; furthermore, these reducing agents react with wool dyes and strip them from the fibers.

An object of the present invention is to provide a method for wet processing of wool and other hair fibers in which the effect of overcoming the yellowish cast will be durable and which will not affect disadvantageously the hand or character of the wool.

Another object is to provide a wet processing system for treating wool and other hair fibers wherein the tendency of the yellowish cast or coloration to increase will be eliminated entirely and on the contrary the fibers will be lightened and brightened.

Other objects of the present invention will become apparent in the course of the following specification.

The present invention is based to a substantial extent on the surprising discovery that a hydroxylamine salt of a strong acid such as the sulfate or chloride, is most effective for this purpose.

Extensive experimentation has shown that hydroxylamine salts of strong acids while being definitely reducing agents, act differently from other conventional reducing agents when applied to animal fibers, such as wool. Hydroxylamine salts were found to have the unique property of lightening and brightening wool and other hair fibers without destroying the dyes. The effect produced is durable and long lasting. Apparently this is caused by the fact that these compounds act only on the wool sub-strata.

According to the present invention the preferred salts are mineral acid salts of hydroxylamine, such as the sulfate and the chloride.

2

In a preferred embodiment of the invention the salt used is hydroxylamine sulfate which is available commercially in highly concentrated form, namely, in 95% to 97% concentration with two mols of hydroxylamine combined with one mol of sulfuric acid.

It was found that hydroxylamine salts may be used in the dye bath together with wool dyes and that one operation is sufficient to accomplish the brightening or whitening of the wool, as well as the dyeing.

This contrasts remarkably with prior art procedures for obtaining bright pale shades of wool in which wool had to be bleached with hydrogen peroxide in a separate operation before dyeing. This operation is not only costly but also has a tendency to damage the wool since it is carried out in an alkaline medium.

According to the present invention the concentration in the bath may vary from 0.015% to 0.5% and the processing may take place at a pH of 2.0 to 7.0.

According to a preferred embodiment hydroxylamine sulfate is used in the amount of from 0.015% to 0.1% of bath volume and at a pH of 3.5 to 4.5.

The use of hydroxylamine sulfate and other mineral acid salts in the dye bath improves the light fastness of the dyed wool.

This treatment minimizes the tendency of the dyed shade to change toward red, commonly referred to as "red fade," when exposed to sunlight or in the Fade-o-meter.

There is, however, a disadvantage in the use of a hydroxylamine salt in the dye bath, in that there is a tendency toward unlevel shades when dyeing pale shades (0.1%—0.25% OWF) with milling or neutral premetalized dyes. These dyes usually have a high rate of exhaustion at a low pH in the range of 3.0—5.0, which is the range usually encountered when hydroxylamine salts are present in the bath. Furthermore, hydroxylamine salts of strong acids are quite corrosive to ordinary steel dyeing kettles and storage containers.

To overcome this corrosive effect it has been found that small amounts of ammonium, sodium and potassium salts of phosphoric acid are very useful in inhibiting corrosion effects resulting from the use of hydroxylamine salts even though the pH of the treating bath be as low as 3.0. These phosphate salts also act as buffers in acid media and furthermore provide level dyeings even in pale shades.

Also it has been found that the use of ammonium silicofluoride or other water soluble silicofluorides in combination with the hydroxylamine salts, enhance the brightening effect on wool or other hair fibers in the dyeing process.

In general, sodium sulfate, sulfuric acid, a silicofluoride and a phosphate may be added to the hydroxylamine for the processing operation.

The following examples are given solely by way of illustration and not by way of limitation.

Throughout the following examples the percentages of chemicals and dyes used in the dye bath are based on the weight of the fiber.

## EXAMPLE I

60 A 30:1 bath was prepared with 10% sodium sulfate, 1% acetic acid (50%), and 4% of the following product:

Parts

65 Hydroxylamine sulfate \_\_\_\_\_ 40

Ammonium silicofluoride \_\_\_\_\_ 20

Disodium phosphate \_\_\_\_\_ 40

100

Scoured wool/worsted fabric was entered at 120° F. and the bath was heated gradually to the boil and the boiling continued for one hour. The bath was cooled, dropped, and the fabric rinsed thoroughly and dried.

A control sample was treated at the same time using the same procedure, but omitting the product of this invention. The sample treated with the product of this invention was much lighter and brighter than the control sample.

#### EXAMPLE II

A 30:1 bath was prepared at 100° F. with 10% anhydrous sodium sulfate, 2% sulfuric acid, and 3% of the following product:

|                       | Parts |
|-----------------------|-------|
| Hydroxylamine sulfate | 50    |
| Disodium phosphate    | 10    |
| Monosodium phosphate  | 40    |
|                       | <hr/> |
|                       | 100   |

Scoured wool/worsted fabric was entered into bath and worked ten minutes at 105° F. Then 0.25% C.I. Acid Blue 45, predissolved, was added and the bath was heated gradually to boiling point and boiled for one hour. Then bath was cooled, dropped and the fabric rinsed thoroughly and dried.

The dyeing is much brighter than the control dyed simultaneously, but without the use of the hydroxylamine composition.

#### EXAMPLE III

A 30:1 bath was prepared at 100° F. with 10% sodium sulfate, 2% ammonium sulfate, and 2% of the following product:

|                         | Parts |
|-------------------------|-------|
| Hydroxylamine sulfate   | 50    |
| Ammonium silicofluoride | 20    |
| Disodium phosphate      | 20    |
| Monosodium phosphate    | 10    |
|                         | <hr/> |
|                         | 100   |

Scoured wool/worsted fabric was entered into bath and worked for ten minutes. Then 0.1% C.I. Acid Blue 80 was added and the bath brought gradually to the boil and the boiling continued for 45 minutes.

The dyeing is much brighter than a control dyeing carried out without above product.

#### EXAMPLE IV

A 25:1 bath was prepared at 100° F. with 5% sodium sulfate, 1% acetic acid (50%), and 1.5% of the following product:

|                         | Parts |
|-------------------------|-------|
| Hydroxylamine sulfate   | 60    |
| Diammonium phosphate    | 20    |
| Monosodium phosphate    | 5     |
| Ammonium silicofluoride | 15    |
|                         | <hr/> |
|                         | 100   |

Prescoured worsted yarn was entered into this bath and run for ten minutes. Then 0.1% C.I. Acid Blue 78 was added to bath and it was gradually heated to boil and boiled for one hour. The bath was then cooled, dropped, the yarn was rinsed thoroughly and dried.

This dyeing is much brighter and clearer than a control dyeing carried out simultaneously.

#### EXAMPLE V

A 25:1 bath was prepared at 105° F. with 10% sodium sulfate, 2% formic acid (90%), and 1% of the following product:

|                          | Parts |
|--------------------------|-------|
| Hydroxylamine sulfate    | 50    |
| Disodium phosphate       | 20    |
| Monosodium phosphate     | 10    |
| Magnesium silicofluoride | 20    |
|                          | <hr/> |
|                          | 100   |

Prescoured carpet yarn was entered into this bath and run for ten minutes. Then 0.1% Brilliant Alizarine Light Blue 3F was added. The bath was brought to a boil and the boiling was continued for 45 minutes. The bath was then cooled, dropped and the yarn rinsed thoroughly and dried.

This dyeing was also brighter and bluer than a control dyeing which was carried out at the same time.

#### EXAMPLE VI

A 30:1 bath was prepared at 100° F. with: 10% sodium sulfate, 2% ammonium sulfate, and 1.5% of the composition described in Example III.

The prescoured wool/worsted fabric was entered and run for ten minutes. Then 0.1% C.I. Acid Brown was added. The bath was heated to 190° F. and the dyeing continued for one hour at this temperature.

The bath was cooled, dropped, and fabric was rinsed thoroughly and dried. The dyed sample was considerably brighter than a control sample.

#### EXAMPLE VII

A 25:1 bath was prepared at 100° F. with: 10% sodium sulfate, 2% ammonium sulfate, and 2% of the composition described in Example II.

Then 0.05% Irgalan Brown Violet DL (Geigy) (no color index designation being available), was added. A fabric consisting of 60% wool/40% mohair was entered and was run for ten minutes. The bath was brought gradually to the boil and the boiling continued for 45 minutes. The bath was then cooled, dropped and the fabric rinsed thoroughly and dried. This fabric was considerably brighter than a control dyeing.

#### EXAMPLE VIII

A 25:1 bath was prepared at 100° F., with 10% sodium sulfate, 2% sulfuric acid, and 2% of the following product:

|                       | Parts |
|-----------------------|-------|
| Hydroxylamine sulfate | 55    |
| Disodium phosphate    | 5     |
| Monosodium phosphate  | 20    |
| Sodium sulfate        | 20    |
|                       | <hr/> |
|                       | 100   |

Scoured worsted yarn was entered and worked in the bath for ten minutes. Then 0.015% C.I. Acid Red I was added and dyeing continued according to Example VII. This dyed sample was considerably brighter than a control.

#### EXAMPLE IX

Scoured wool flannel was entered into a 30:1 bath which contained 10% sodium sulfate, 2% formic acid (90%), and 1% of the following product:

|                        | Parts |
|------------------------|-------|
| Hydroxylamine chloride | 75    |
| Monosodium phosphate   | 20    |
| Disodium phosphate     | 5     |
|                        | <hr/> |
|                        | 100   |

After running for ten minutes, 0.1% C.I. Acid Blue 78 was added and the dyeing continued as in Example VII. Resulting dyeing was brighter than the control.

#### EXAMPLE X

Peroxide bleached wool vs. wool treated as in Example III.

(a) A piece of scoured wool/worsted flannel was subjected to a full bleach as follows: A 25:1 bath was prepared at 140° F. with a 0.25% (on weight of bath) tetrasodium pyrophosphate and three volumes of hydrogen peroxide. Flannel was entered and was bleached for two

hours at this temperature. Flannel was rinsed thoroughly, neutralized with 2% (OWF) acetic acid (50%) and then dried.

(b) Another piece of above flannel was treated as follows: a 25:1 bath was prepared at 105° F. with 10% sodium sulfate, 1% (OWF) acetic acid, and 3% of the product of Example III.

Bath was brought to boil and boiled for one hour. The bath was cooled, then dropped and fabric rinsed thoroughly and dried.

(c) A piece of the same flannel was treated as in (b) except that the hydroxylamine of Example III was omitted. Sample (b) was much whiter than sample (c), although not as white as sample (a).

When all three samples were exposed to 40 hours in the Fade-o-meter, the bleached sample (a) acquired about the same yellow color as the unbleached sample (c). Sample (b) yellowed only imperceptibly.

#### EXAMPLE XI

A 30:1 bath was prepared at 110° F. with 10% sodium sulfate, 4% sulfuric acid, and 1% of product of Example VIII.

Scoured carpet yarn was entered into bath and was worked in the bath for ten minutes. Then 0.1% C.I. Acid Blue 158 (A.M.) was added. The bath was brought to boil within 25 minutes and the boiling continued for 45 minutes. The bath was then cooled, dropped and the yarn rinsed thoroughly and dried. The dyed yarn was considerably brighter than a control dyeing which was dyed without hydroxylamine.

What is claimed is:

1. A method of wet processing wool and other hair fibers, which comprises processing the hair fibers in the

presence of hydroxylamine which is in the form of a strong mineral acid at a pH of 2.0 to 7.0 in amounts from 0.015% to 0.5% of the bath.

2. A method of wet processing wool and other hair fibers in accordance with claim 1, wherein the processing also takes place in the presence of a water soluble silicofluoride and a alkali metal phosphate.

3. A method of wet processing wool and other hair fibers in accordance with claim 1, wherein the processing also takes place in the presence of sodium sulfate, sulfuric acid, a silicofluoride and a phosphate.

4. Wool fibers treated in accordance with the method described in claim 1.

5. A method of wet processing wool and other hair fibers, which comprises processing the hair fibers in the presence of hydroxylamine sulfate in the amount of from 0.015% to 0.1% of bath volume at a pH of 3.5 to 4.5.

6. A method of wet processing wool and other hair fibers in accordance with claim 5, wherein the processing also takes place in the presence of a silicofluoride using 4 to 5 parts and an alkali metal phosphate using 4 to 10 parts, to 10 parts of the hydroxylamine sulfate.

#### References Cited

##### UNITED STATES PATENTS

|           |         |                 |       |            |
|-----------|---------|-----------------|-------|------------|
| 2,382,632 | 8/1945  | Hessel et al.   | ----- | 8—127.6    |
| 2,545,450 | 3/1951  | Dalton et al.   | ----- | 8—127.6 XR |
| 3,282,639 | 11/1966 | Lundgren et al. | ----- | 8—127.6    |

MAYER WEINBLATT, Primary Examiner.

U.S. CL. X.R.

8—107, 128, 133